

# UNITED STATES PATENT OFFICE.

ROBERT MUH AND ALBERT SCHUPP, OF LOCH SHELDRAKE, NEW YORK.

ROAD-SURFACING COMPOSITION FOR SURFACING ROADS, DRIVEWAYS, AND SIDEWALKS.

1,074,131.

Specification of Letters Patent. Patented Sept. 30, 1913.

No Drawing.

Application filed April 10, 1913. Serial No. 760,187.

*To all whom it may concern:*

Be it known that we, ROBERT MUH and ALBERT SCHUPP, citizens of the United States, residing at Loch Sheldrake, in the county of Sullivan and State of New York, have invented certain new and useful Improvements in Road-Surfacing Composition for Surfacing Roads, Driveways, and Side-walks, of which the following is a specification.

Our composition consists of the following ingredients, combined in the proportions stated, viz:—refined Bermudaz asphalt, four pounds; #1 stearin pitch, one pound; ordinary dirt, eight pounds; cement, four pounds. These ingredients are to be thoroughly mixed and combined as follows:—The asphalt is boiled, and when it has reached the boiling point the other ingredients are mixed in, and with, the boiling asphalt, and when they are thoroughly combined by agitation, the composition is placed upon the prepared surface of the road, drive-way, or side walk to the thickness of 25 from one-half inch to one inch in thickness in proportion to the demands of travel over the way thus surfaced.

By the use of the above composition, properly prepared and applied, and allowed to cool and set firm before being traveled over, we secure a smooth, firm, and durable road surface at a moderate cost.

While it may be claimed that each of the ingredients mentioned have at some time, and in some way, been used for similar purposes, yet we are not aware that all of the ingredients in our composition have been used in the proportions, and in the manner described.

We claim:—

1. The herein described composition of matter consisting of refined Bermudaz asphalt; #1 stearin pitch; ordinary dirt; and cement containing about equal amounts of asphalt and cement, more dirt than cement or asphalt, and less stearin pitch than cement or asphalt, substantially as described, and for the purposes specified. 40

2. The herein described composition of matter for surfacing of roads, drive-ways, and sidewalks, consisting of refined Bermudaz asphalt, four pounds; #1 stearin pitch, one pound; ordinary dirt, eight pounds; and cement, four pounds, substantially as described. 50

In testimony whereof we affix our signatures in presence of two witnesses.

ROBERT MUH.  
ALBERT SCHUPP.

Witnesses:

LENA BRENNER,  
ELSWORTH BAKER.